

## 1

3,089,848  
OIL COMPOSITIONS CONTAINING  
SODIUM NITRITE

Arnold J. Morway, Clark, N.J., assignor to Esso Research and Engineering Company, a corporation of Delaware  
No Drawing. Filed May 5, 1960, Ser. No. 26,964  
9 Claims. (Cl. 252—18)

This invention relates to lubricating compositions containing sodium nitrite as a rust preventive. Particularly, the invention relates to compositions wherein the effectiveness of sodium nitrite is enhanced by certain auxiliary additives and to methods whereby sodium nitrite is dispersed in stable, finely divided form, in lubricating greases.

The use of sodium nitrite as a rust preventive has long been recognized and it has been proposed to add sodium nitrite to lubricating greases in order to inhibit rusting of metal surfaces. This rusting can be caused by water or moisture which may become absorbed or entrained in the grease during use or actually rejected by water repellent greases, thus directly contacting metal surfaces.

It has now been found that the use of certain auxiliary additive materials, specifically, metal naphthenates and fatty acid partial esters of aliphatic polyhydric alcohols (e.g. sorbitan monooleate), will increase the effectiveness of the sodium nitrite in preventing rust much more than would be expected.

In addition, a new method of dispersing sodium nitrite in grease has also been found, which overcomes many of the disadvantages of prior methods. One such prior method involved mixing an aqueous solution of sodium nitrite into the lubricating grease and then heating to evaporate the water to thereby obtain a homogeneous dispersion of the nitrite in the grease. However, if the grease contains a soap or salt of a metal other than sodium, particularly divalent metals, then metathesis occurs at the high temperature necessary for the evaporation of water. The result is that metal of the soap or salt thickener is exchanged by sodium, thereby changing the characteristics of the original grease. This has been found particularly objectionable in the manufacture of alkaline earth metal greases, e.g. calcium soap grease, since the structural stability of the grease is down-graded by metathesis with the sodium nitrite. Another disadvantage of this method is that sodium nitrite crystallizes out of the aqueous solution in the form of rather large particles or crystals. These particles give the grease a grainy texture, as well as increasing its wearing tendency due to the abrasive nature of the sodium nitrite particles. Even when increased wear is not too great, the large size crystals give noisy and objectionable anti-friction bearing operation.

Another prior method of dispersing sodium nitrite in grease is disclosed in U.S. Patent No. 2,738,329. Here, the grease with sodium nitrite present, is heated to form a hot, fluid composition, i.e. heated to a temperature above the melting point of the grease. Upon cooling of the composition, the dropping point of the grease was very materially increased and other changes effected, even by the addition of small amounts of sodium nitrite. Apparently, some form of complex was formed between the grease thickener and the sodium nitrite. Thus, this method is not applicable where the aim is only to increase the rust resistance of the grease, but not to alter any of its other properties.

## 2

Another prior method involves the simple addition of powdered sodium nitrite into a finished grease composition with stirring. This method, even though the resulting composition is homogenized, results in a grainy grease, increases its wearing tendency and frequently causes noisy bearing operation.

In the method of the present invention, sodium nitrite can be added to a grease without affecting any of the other properties of the grease except inhibiting rusting caused by entrained water. Furthermore, a smooth, homogeneous, non-grainy product is obtained.

In the preferred form of the present method, commercial granular sodium nitrite is first dissolved in water, preferably boiling water, to form a super-saturated solution. Then a water gelling agent is added to gel the solution which will thereby inhibit growth of any crystals that may form. Next, this water gel is mixed with an oil solution containing a low molecular weight polymer and the entire mixture is then heated to drive off the water. As the water evaporates, the sodium nitrite crystals which are forming are coated by the low molecular weight polymer and their crystal growth is inhibited. The result is an oil dispersion of very finely divided sodium nitrite. This oil dispersion may then be conveniently mixed into the final grease composition, since the sodium nitrite concentrate dispersion is readily dispersed in cold or warm grease compositions with a minimum of mixing.

The sodium nitrite is used in the final grease composition in amounts of 0.1 to 3.0 wt. percent, preferably 0.3 to 1.0 wt. percent, based on the weight of the total composition. The auxiliary additives which increased the effectiveness of the sodium nitrite are used in amounts of 0.05 to 1.0 part by weight, per part by weight of sodium nitrite.

The naphthenates are preferably the zinc or sodium salts of naphthenic acids, preferably having molecular weights of 250 to 350 and neutralization numbers of 225 to 175.

The fatty acid partial ester materials include the C<sub>12</sub> to C<sub>22</sub> fatty acid partial esters of aliphatic polyhydric alcohols having about 3 to 12, e.g., 3 to 8 carbon atoms, and about 2 to 8, e.g., 3 to 6 hydroxy groups per molecule. Preferred materials are the mono- and diesters of C<sub>3</sub> to C<sub>6</sub> alcohols having about 3 to 6 hydroxyl groups and prepared from C<sub>12</sub> to C<sub>18</sub> fatty acids. The above type of partial esters includes the partial esters of the mono-hydrated aliphatic polyhydric alcohols, which are well known in the art, for example, see U.S. Patent 2,434,490, as well as partial esters of non-dehydrated aliphatic polyhydric alcohols, e.g. pentaerythritol monooleate.

Specific examples of the above types of partial esters will therefore include: glyceryl monooleate, pentaerythritol monooleate, sorbitan monooleate, the dioleates of sorbitan, mannan, pentaerythritol and related polyhydric alcohols, the corresponding partial stearic and palmitic acid esters of these alcohols, and partial esters of these alcohols made from mixtures of these fatty acids.

The rust inhibiting combination may be added to any type of grease composition. Included are greases thickened with salts, soaps, soap-salt or mixed salt complexes, polymeric thickeners (e.g. polymers of C<sub>2</sub> to C<sub>4</sub> monolefins of 10,000 to 200,000 molecular weight such as polyethylene), and inorganic thickeners (e.g. clay, carbon black, silica gel, etc.).

Generally, the greases will comprise either a synthetic or mineral lubricating oil thickened with about 3 to 35 wt. percent, usually 3 to 20 wt. percent, of a thickener. In the case of soap-salt and mixed-salt thickeners, the thickener is usually formed by co-neutralization in oil, by metal base, of various mixtures of high molecular weight fatty acids and/or intermediate molecular weight fatty acids with low molecular weight fatty acids.

The high molecular weight fatty acids useful for forming soap-salt, soap and mixed-salt thickeners include naturally-occurring or synthetic, substituted and unsubstituted, saturated and unsaturated, mixed or unmixed fatty acids having about 14 to 30, e.g. 16 to 22, carbon atoms per molecule. Examples of such acids include stearic, hydroxy stearic, such as 12-hydroxy stearic, di-hydroxy stearic, poly-hydroxy stearic and other saturated hydroxy fatty acids, arachidic, oleic, ricinoleic, hydrogenated fish oil, tallow acids, etc.

Intermediate molecular weight fatty acids include those aliphatic, saturated, unsubstituted, mono-carboxylic acids containing 7 to 12 carbon atoms per molecule, e.g., capric, lauric, caprylic, nonanoic acid, etc.

Suitable low molecular weight acids include C<sub>2</sub> to C<sub>4</sub> fatty acids. Acetic acid or its anhydride is preferred.

Metal bases which are frequently used to neutralize the above acids are the hydroxides, oxides or carbonates of alkali metals (e.g. lithium and sodium) or of alkaline earth metals (e.g. calcium, magnesium, strontium and barium).

Various other additives may also be added to the lubricating composition (e.g. 0.1 to 10.0 weight percent based on the total weight of the composition), for example, oxidation inhibitors such as phenyl-alpha-naphthylamine; tackiness agents such as polyisobutylene; stabilizers such as aluminum hydroxy stearate; and the like.

As previously mentioned, the sodium nitrite and the other additives are preferably added to the grease in such a way so as to obtain an extremely small particle size. This is best accomplished by dissolving about 40 to 60 wt. percent based on total weight of water solution, of the combined sodium nitrite and auxiliary enhancing agent in water. Preferably as little water as possible is used to minimize the amount to be later removed by evaporation. This can be accomplished by using hot water, e.g. 150-212° F., preferably boiling water. Into this hot water solution, and preferably as quickly as it is formed and before any crystallization can occur, about 0.1 to 1.0 wt. percent, based on total weight of water solution, of a water gelling agent is added. The water gelling agent thickens or gels the solution upon cooling to substantially immobilize the solution. Thus, any sodium nitrite which crystallizes out from the solution is inhibited from growing into larger crystal sizes. Any water gelling or water thickening agent may be used. Preferred are the various ether celluloses such as methyl cellulose, ethyl cellulose or a group of materials sold under the tradename of Jaguar resins. Jaguar is Stein-Hall's registered trademark for guar gum, a natural vegetable colloid. Guar gum is a polysaccharide (chemically classified as a galactomannan) consisting of a complex carbohydrate polymer of galactose and mannose. It is non-ionic and therefore will not gel in the presence of ionic salt solutions. Another particularly useful material to prevent the growth of crystals is a carboxy vinyl polymer neutralized with sodium hydroxide. A material of this type which was used in several of the examples is Carbopol 934 which has been neutralized with sodium hydroxide by simple mixing without removing the water of neutralization.

The above described water dispersion, either hot or cold, is next mixed with about .25 to 2.0 parts by weight, per part of water solution, of an oil solution of a polymeric material. Preferably polymers having molecular weights of about 5,000 to 100,000 and which are oil dispersible can be used. Preferred polymers of this type are polypropylene and polyethylene, i.e. C<sub>2</sub> to C<sub>3</sub> monoolefin poly-

mers. Such polymers are used in amounts of .05 to .15 part by weight, per part by weight of oil.

Next, the combination of the water solution and oil solution is heated sufficiently to drive off substantially all the water. The result is a stable oil dispersion of the sodium nitrite in a very finely divided form dispersed in the oil. This oil solution in turn can be added to any grease composition.

While the above technique represents a preferred method of preparing the compositions of the invention, it is to be understood that the naphthenates and/or partial esters may be used with the sodium nitrite employing other methods to disperse the nitrite in oil. For example, just simple mixing of finely divided sodium nitrite and the naphthenate and/or partial ester into the grease will give better rust protection than a like amount of either material alone. This simple mixing will result in a grainy grease giving noisy bearing operation as previously mentioned. However, while less preferred, this method may be used when graininess or noisy bearing operation are not important considerations.

The invention will be further understood by the following examples:

#### EXAMPLE I

(All parts by weight)

*Inhibitor concentrate 1.*—50 parts of sodium nitrite was dissolved in 50 parts of hot water while maintaining a temperature of 210° F. 0.5 part of Carbopol 934 (carboxy vinyl polymer) neutralized with sodium hydroxide in 0.2 part of water was next added, while boiling the sodium nitrite aqueous solution. After all the neutralized Carbopol 934 had been added and while still boiling the solution, there was next added 50 parts of an oil dispersion consisting of 10 wt. percent of atactic polypropylene having an average molecular weight of about 50,000, 1 wt. percent Span 80 (sorbitan monooleate) and 89 wt. percent of a mineral lubricating oil having a viscosity of 55 SUS at 210° F. Boiling of the entire mixture was continued until all the water had been removed. The resulting dispersion had the following composition:

|                               | Percent |
|-------------------------------|---------|
| Sodium nitrite                | 49.5    |
| Neutralized Carbopol 934      | 0.5     |
| Atactic polypropylene         | 5.0     |
| Span 80 (sorbitan monooleate) | 0.5     |
| Mineral oil                   | 44.5    |

*Inhibitor concentrate 2.*—The above preparation was repeated to form a second inhibitor concentrate but which contained no Span 80 whatsoever and instead contained 50.0 wt. percent sodium nitrite.

*Inhibitor concentrate 3.*—A third inhibitor concentrate was prepared by dispersing 50 wt. percent of sodium nitrite in 50 wt. percent of a mineral oil having a viscosity of 55 SUS at 210° F. The sodium nitrite used was one of the most finely divided sodium nitrites available having an average particle size of about 35 microns.

Portions of each of the above inhibitor concentrates 1 to 3 were added by simple mixing at room temperature, in the amounts of 1, 2, 3 and 4 wt. percent, respectively, based on the weight of the total composition, to a calcium salt grease.

The calcium salt grease was prepared by neutralizing with lime, a mixture of acetic acid and Wecoline AAC acids (a mixture of C<sub>8</sub>, C<sub>10</sub> and C<sub>12</sub> fatty acids having an average molecular weight of about 170). The neutralized mixture of acids was heated to a temperature of about 440° F. and dehydrated. About 6 moles of acetic acid were used per mole of Wecoline AAC acid. The total amount of thickener constituted about 22 wt. percent of the grease, while its oil base was a mineral lubricating oil of 55 SUS viscosity at 210° F. After cooking at a temperature of 440° F. the grease was cooled to about

200° F. and about 1 wt. percent of phenyl-alpha-naphthylamine added as an oxidation inhibitor, following which the grease was homogenized in a Charlotte colloid mill.

These grease compositions containing the various inhibitor concentrates were tested by the CRC L-41 procedure which is an ASTM Tentative Method of Test for: Rust Preventive Properties of Lubricating Greases. Briefly stated this procedure involves taking a clean small Timken roller bearing, coating and packing the bearing with grease, rotating the bearing at 1750 r.p.m. under a load of 6 lbs. for one minute, then dipping the bearing in freshly boiled distilled water, followed by storing the bearing over water in a sealed jar for 14 days so as to provide a humid atmosphere. At the end of 14 days the bearing is cleaned and examined for rust. The bearing is then rated on a scale, wherein R-1 represents no rust whatsoever, R-2 represents no more than 2 faint rust spots, and R-3 represents more than 2 faint rust spots. R-3 is considered a complete failure, while R-1 and R-2 are considered as passing. Bearings having large rust spots were considered as failing badly.

The compositions prepared above, including the base grease without any rust preventive whatsoever, were tested by the above procedure. The results obtained are summarized in the following table:

Table I  
RESULTS OF CRC L-41 RUST TEST

| Amount Inhibitor Concentrate Added | Type Inhibitor Concentrate |            |             |
|------------------------------------|----------------------------|------------|-------------|
|                                    | 1                          | 2          | 3           |
| None *                             |                            |            |             |
| + 1%                               | Pass R-2                   | Fail Badly | Fail Badly. |
| 2%                                 | do                         | do         | Do.         |
| 3%                                 | Pass R-1                   | Fail R-3.  | Fail R-3.   |
| 4%                                 | do                         | Pass R-1   | Pass R-1.   |

\* The grease without inhibitor failed badly.

1. Contains oil, sodium nitrite, neutralized Carbopol 934, polypropylene and Span 80.

2. Contains oil, sodium nitrite, neutralized Carbopol 934, polypropylene, (no Span 80).

3. Simple oil concentrate of sodium nitrite.

As seen by the above table, the compositions containing both the sodium nitrite and Span 80 (inhibitor concentrate 1) were very successful in the corrosion test even when used in an amount as low as 1 weight percent of inhibitor concentrate. On the other hand, by leaving out the extremely small amount of Span 80 involved, it required 4% of the inhibitor concentrate in order to effectively inhibit the rusting as shown by the results obtained when using inhibitor concentrates 2 and 3.

A second grease was prepared and all of the above tests repeated. The second grease was formed by neutralizing 13 parts of hydrated lime with 15.1 parts of acetic anhydride and 9.4 parts of Emery 32865 acid (a treated vegetable fatty acid consisting mainly of iso-oleic acid) in 61.5 parts of mineral lubricating oil having a viscosity of 55 SUS at 210° F., to which was added one part of phenyl-alpha-naphthylamine, (all parts are by weight). The neutralized mixture was dehydrated at a temperature of about 300° F. Exactly the same results were obtained with the second grease as were reported in Table I.

#### EXAMPLE II

A base grease was prepared (wherein all parts are by weight), by dispersing 9.4 parts of tallow fatty acids and 13 parts of hydrated lime in 61.5 parts of mineral lubricating oil having a viscosity of 55 SUS at 210° F. These materials were mixed together at room temperature, and while stirring, 15.1 parts of acetic anhydride was slowly added, the temperature rising to a maximum of 180° F. After all the anhydride was added, external heating was initiated and the temperature of the composition increased to 320° F. in order to dehydrate the grease. At this

point, 1 part of phenyl-alpha-naphthylamine was added as an oxidation inhibitor and the grease was allowed to cool to 90° F. The grease was then passed through a Morehouse mill having an 0.003" clearance. The resulting product had a dropping point above 500° F. and an ASTM unworked penetration at 77° F. of 323 mm./10, which upon working 10,000 strokes decreased only to 319 mm./10. The grease was also insoluble in both hot and cold water.

To the above base grease, was added sodium nitrite having an average particle size of 35 microns and zinc naphthenate in varying amounts. The zinc naphthenate was the zinc salt of a 250 molecular weight naphthenic acid obtained from a petroleum diesel oil fraction. These two materials were incorporated by mixing directly into the grease and then twice homogenizing in a Morehouse mill in order to thoroughly disperse the additive in the grease. Other samples were made up using the sodium nitrite and naphthenate alone. These various samples were then subjected to CRC L-41 test procedure described above. The results obtained are summarized in the following table:

Table II  
RUST TESTS—CRC L-41 PROCEDURE

|                              | Amount of Additive <sup>1</sup> | Results of Rust Test                             |
|------------------------------|---------------------------------|--------------------------------------------------|
| None                         |                                 | Fail (R-3), Badly rusted.                        |
| 1% Zinc Naph.                |                                 | Fail (R-3).                                      |
| 2% Zinc Naph.                |                                 | Badly rusted.                                    |
| 2% NaNO <sub>2</sub> (35μ)   |                                 | Pass (R-1), Unaffected, no rust spots or stains. |
| 1.0% NaNO <sub>2</sub> (35μ) |                                 | Fail (R-3), Badly rusted.                        |
| 0.5% NaNO <sub>2</sub> (35μ) |                                 | Pass (R-1), Excellent protection.                |
| 0.25% Zinc Naph.             |                                 |                                                  |

35 1 Wt. percent based on the weight of the total composition.

As shown by the above table, the base grease failed badly in the rust test and still failed upon the addition of up to 2 wt. percent zinc naphthenate and up to 1% sodium nitrite. However, it was found that a mixture of 0.5% sodium nitrite and 0.25% of zinc naphthenate was quite effective, even though much larger amounts of either material alone gave rust. The obvious advantage of the combination is that a smaller overall amount of rust preventive additive is needed.

#### EXAMPLE III

A colloidal sodium nitrite concentrate base was prepared in the same general manner described above in Example I. The finished concentrate had the following composition:

| Composition of concentrate:                 | Percent wt. |
|---------------------------------------------|-------------|
| Water                                       | 2.00        |
| Sodium nitrite                              | 49.0        |
| Carbopol 934 (neutralized)                  | 0.13        |
| Span 80                                     | 0.05        |
| Atactic polypropylene                       | 5.00        |
| Mineral oil of 55 SUS, viscosity at 210° F. | 43.82       |

This concentrate was prepared as follows:

60 The sodium nitrite was added to an equal amount by weight of water and the mixture heated to boiling to completely dissolve all the nitrite. To this hot saturated aqueous solution was added a dispersion of Carbopol 934 dispersed in an amount of water equal to 1/2 the amount of water used in dissolving the sodium nitrite. After all 65 the dispersion of Carbopol 934 had been added to the boiling water solution of sodium nitrite, and while still boiling, an oil solution of polypropylene was added. This polypropylene had a molecular weight of about 50,000. Evaporation of water was continued until about only 2 70 wt. percent of the total composition was water, after which the material was cooled and homogenized in a Morehouse mill at 0.003" clearance. This small amount of water present is desirable since it allows easier handling, results in smaller particle sizes and later gives

greater dispersion of the inhibitor concentrate in the oil. However, if desired, the inhibitor concentrate could be evaporated to complete dryness.

Four grease compositions were prepared in the same general manner as in Example II, but using the inhibitor concentrate described immediately above. The compositions of these greases are summarized in the following table along with their properties:

substantially all of said water to thereby form a dispersion in said oil of polymer-coated sodium nitrite having an average particle size less than about 15 microns.

3. A method according to claim 2, wherein said olefin polymer is polypropylene.

4. A method of dispersing sodium nitrite in an oil which comprises forming a solution of about 40 to 60 wt. percent, based on the weight of said solution, of so-

Table III

| Formulation (Percent Weight)                                                            | Grease A         | Grease B         | Grease C    | Grease D         |
|-----------------------------------------------------------------------------------------|------------------|------------------|-------------|------------------|
| Acetic Acid                                                                             | 10.0             |                  | 12.9        | 12.9             |
| Acetic Anhydride                                                                        |                  | 14.0             |             |                  |
| Wecoline AAC Acid                                                                       | 5.0              |                  | 3.9         | 3.9              |
| Tallow fatty acid                                                                       |                  | 8.7              |             |                  |
| 12-hydroxy stearic acid                                                                 | 0                | 0                | 2.0         | 2.0              |
| Hydrated lime                                                                           | 8.3              | 12.0             | 8.6         | 8.6              |
| Phenyl- <i>n</i> -naphthylamine                                                         | 1.0              | 1.0              | 0.3         | 0.3              |
| Mineral oil                                                                             | 71.7             | 60.3             | 71.9        | 67.9             |
| NaN <sub>3</sub> Concentrate                                                            | 4.0              | 4.0              | 0.0         | 4.0              |
| Appearance                                                                              | Excellent        | Excellent        | Excellent   | Excellent        |
| Dropping Point, °F.                                                                     | 500              | 500+             | 500+        | 500+             |
| Penetrations, 77° F., mm./10:                                                           |                  |                  |             |                  |
| Unworked                                                                                | 320              | 310              | 271         | 269              |
| Worked 60 strokes                                                                       | 330              | 315              | 291         | 298              |
| Worked 10,000 strokes                                                                   | Semi-Fluid       | 317              | 304         | 377              |
| Rust Tests: CRC L-41 Method, Rating                                                     | R-1 (No rusting) | R-1 (No rusting) | R-3 (Fails) | R-1 (No rusting) |
| Microscopic examination determination of particle size of the sodium nitrite in microns | About 10         | About 10         | About 10    | About 10         |

As seen by the above table, grease C which contained no sodium nitrite failed in the rust test, while greases A, B and D gave no rusting and had good all around properties. Furthermore, the preferred method of the invention resulted in sodium nitrite particles of about 10 micron size, while other common methods of forming sodium nitrite crystals result in larger particle size. Thus, the method can give particle sizes of 15 microns or less, while commercial sodium nitrite is of about 35 micron size. Simple evaporation of aqueous solutions of sodium nitrite in oil will also give a micron size of 35 or higher. As mentioned above, such larger particles (i.e. about 35 microns) give a gritty texture to the grease and causes noisy bearing operation which is avoided by the method of the invention.

In summary, the present invention primarily relates to additive combinations of sodium nitrite with zinc or sodium naphthenate and/or certain partial esters. The invention further relates to a new method of forming finely divided sodium nitrite in oil. The additive combinations are best used in the form of oil concentrates comprising about 20 to 60 wt. percent additive and 80 to 40 wt. percent oil, preferably mineral oil, although of course any less amount of additive in oil can be used.

What is claimed is:

1. A method of forming a stable dispersion of finely divided sodium nitrite in oil, said dispersion being useful as a rust preventive additive, which comprises forming a solution of sodium nitrite in water, adding to said solution a water gelling agent to gel said solution to thereby inhibit crystal growth of said sodium nitrite, adding to said solution an oil solution of an oil-soluble hydrocarbon polymer having a molecular weight of from about 5,000 to 100,000 to coat said sodium nitrite, heating the resulting mixture to evaporate substantially all of said water to thereby form a dispersion in said oil of polymer-coated sodium nitrite having an average particle size less than about 15 microns.

2. A method of forming a stable dispersion of finely divided sodium nitrite in oil, said dispersion being useful as a rust preventive additive, which comprises forming a solution of sodium nitrite in water, adding to said solution a water gelling agent to gel said solution to thereby inhibit crystal growth of said sodium nitrite, adding to said solution an oil solution of a C<sub>2</sub> to C<sub>3</sub> olefin polymer of 5,000 to 100,000 molecular weight to coat said sodium nitrite, heating the resulting mixture to evaporate

30 sodium nitrite in boiling water; adding about 0.1 to 1.0 wt. percent, based on the weight of said solution, of a water gelling agent to the boiling water solution of sodium nitrite to thereby inhibit crystal growth of said sodium nitrite; adding to the resulting water solution, about 0.25 to 2.0 parts by weight, per part by weight of water solution, of an oil solution comprising 5 to 15 wt. percent of a C<sub>2</sub> to C<sub>3</sub> olefin polymer of 5,000 to 100,000 molecular weight, heating the resulting mixture to evaporate substantially all of said water to thereby form a dispersion in said oil of sodium nitrite having an average particle size less than about 15 microns.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105

a material selected from the group consisting of zinc and sodium salts of naphthenic acid of 200 to 350 molecular weight and  $C_{12}$  to  $C_{22}$  fatty acid partial esters of  $C_3$  to  $C_{12}$  aliphatic polyhydric alcohols having 3 to 6 carboxy groups and heating the resulting mixture to evaporate substantially all of said water to thereby form a dispersion in said oil of sodium nitrite having an average particle size less than about 15 microns. 5

## References Cited in the file of this patent

10

## UNITED STATES PATENTS

- |           |                     |                |
|-----------|---------------------|----------------|
| 2,455,659 | Duncan et al. ----- | Dec. 7, 1948   |
| 2,652,361 | Woods et al. -----  | Sept. 15, 1953 |
| 2,716,634 | Black et al. -----  | Aug. 30, 1955  |

|                      |               |
|----------------------|---------------|
| Kroenig et al. ----- | Jan. 24, 1956 |
| Parry et al. -----   | Mar. 13, 1956 |
| Cooke et al. -----   | Aug. 14, 1956 |
| Blake -----          | Dec. 19, 1961 |

## FOREIGN PATENTS

|                     |               |
|---------------------|---------------|
| Great Britain ----- | July 10, 1957 |
| Canada -----        | Nov. 11, 1958 |

## OTHER REFERENCES

Hollabaugh et al.: "Carboxymethylcellulose . . . Uses and Applications," in Industrial and Engineering Chemistry, vol. 37, No. 10, October 1945, p. 946 relied on.